

E. H. NUTTER & T. J. HOOVER.  
METHOD AND APPARATUS FOR ORE CONCENTRATION.  
APPLICATION FILED SEPT. 25, 1911.

Patented Apr. 14, 1914

1,093,463.

Fig. 1.



Fig. 2.



Fig. 3.



# UNITED STATES PATENT OFFICE.

EDWARD HOIT NUTTER, OF NEW YORK, N. Y., AND THEODORE JESSE HOOVER, OF LONDON, ENGLAND, ASSIGNEES TO MINERALS SEPARATION LIMITED, OF LONDON, ENGLAND.

## METHOD AND APPARATUS FOR ORE CONCENTRATION.

1,093,463.

Specification of Letters Patent. Patented Apr. 14, 1914.

Application filed September 25, 1911. Serial No. 651,188.

*To all whom it may concern:*

Be it known that we, EDWARD HOIT NUTTER and THEODORE JESSE HOOVER, citizens of the United States of America, residing, respectively, in the city of New York, county and State of New York, United States of America, and London, England, have invented certain new and useful Improvements in Methods and Apparatus for Ore Concentration, of which the following is a specification.

This invention is for improvements in or relating to a method and apparatus for ore concentration.

Several processes are known in which certain particles are raised to the surface of a liquid containing powdered ore in suspension, by means of bubbles of air or gas that have been caused to attach themselves to these certain particles which are thereby caused to float, while other particles are not so floated. Thus the powdered ore mixed with water containing a mineral-frothing agent may be agitated so as to beat air into the liquid and form a coherent froth by which certain constituents of the ore such as metallic sulfids are floated.

One object of this invention is to improve the apparatus used in this type of process, and apparatus constructed in accordance with this invention is applicable for use in any of the well known froth flotation processes of ore concentration.

In apparatus at present in use in which a mineral bearing froth is formed and collected it is customary for the froth to be removed from the main pulp after the froth has reached a free air surface so that if the gaseous bubbles or some of them burst on reaching the free air surface there is a possibility that some of the mineral contents of the froth will fall back into the pulp or circuit liquor and fail to be separated and this does in fact occur with tender froths from which the mineral has a tendency to shower.

According to this invention a method of ore concentration by the formation of a mineral bearing froth consists in causing the froth as it is formed to fall over a trap, baffle or wall below the level of the free air surface whereby the froth is collected and removed from the pulp before the bubbles can burst.

An apparatus for concentrating ores by gaseous flotation of certain mineral particles in liquid according to this invention comprises the combination with an agitating vessel in which the liquid containing a mineral frothing agent and containing powdered ore in suspension is agitated so as to beat air into it, of a conduit through which the froth passes and a "trap" to catch the froth before or as the bubbles reach a free air surface whereby the froth is collected and removed from the pulp. Thus the conduit through which the froth is caused to pass may have a wall, partition, or lip the top of which is below the normal surface of the froth or at any rate below the free air surface of the froth whereby the froth falls over the wall or lip and is trapped before the bubbles in the froth can burst so that the mineral contents of the bubbles which burst are discharged into the trap compartment and not into the pulp. It is possible to arrange that the froth passes directly out of the mixing vessel and over a lip or trap which is below a free air surface and over which the froth passes whereby the froth is collected immediately after it is formed and removed from the pulp before the bubbles can reach the free air surface and burst.

A feature of this invention consists in the combination with two or more mixing vessels of a passage or separate compartment through which the ore pulp travels in passing from one vessel to the other and a froth conduit from said passage or compartment so that the froth is led away and trapped while the pulp is passing from one vessel to another. A practical form of this apparatus comprises a number of mixing and separating vessels substantially on the same level. Passages outside the vessels or separate intermediate compartments connect each vessel with the adjacent vessel and a froth conduit and trap are arranged at each passage or intermediate compartment whereby the froth formed at each stage of the agitation is led away and trapped while the pulp passes through the series of mixing vessels, passages or compartments. The mixing vessels may be connected together in pairs by orifices in the partitions between them, and the passages outside the vessels may be arranged to connect one vessel of

each pair with the adjacent vessel of the next pair, a froth trap being placed at each passage.

In any of the arrangements described above this invention includes the combination with a first lip which is below the free air surface and over which the whole froth passes into a trap of a second lip over which the more permanent froth passes from the trap into a launder or other collector, and various arrangements may be used for removing the concentrates that sink to the bottom of the trap compartment.

In the accompanying drawings which illustrate by way of example one form of apparatus embodying this invention, Figure 1 is a front elevation partly in section; Fig. 2 is a transverse section, and Fig. 3 is a plan of the apparatus.

Several mixing vessels A are placed side by side on the same level. Each vessel is provided with a rotatable agitator or stirrer A<sup>1</sup> carried by a vertical spindle A<sup>2</sup> rotated at high speed by any convenient means. The first vessel is connected with the second, the second to the third, the third to the fourth and so on by passages or compartments B between the mixing vessels and on the same level with them. By this arrangement the pulp passes from the first vessel A through the connecting passage or compartment B to the second vessel A and so on and at the end of the series the pulp may conveniently be passed into a spitzkasten as described in the previous patent to Hoover, No. 953,746, of April 5, 1910.

At each connecting passage or compartment B there is a froth trap, that is to say baffles or conduits are so arranged in connection with these passages that the mineral-bearing bubbles in rising are directed into a separate compartment from that through which the main circuit passes, before the bubbles reach the free air surface and have a chance to break. Thus, for example, the wall of each connecting passage B may be formed by a partition D the top or lip D<sup>1</sup> of which is below the level of the free air surface of the froth when the apparatus is working.

The froth rises in the connecting passage B and a roof or cover E is provided to lead the froth over the lip or partition D before the bubbles get to a free air surface.

Outside the lip or partition is a trap compartment F into which the mineral-bearing froth falls or passes. The froth reaches a free air surface in this trap compartment F and the bubbles which burst deposit the mineral in the trap compartment. The outer wall G of the trap compartment may comprise a second lip G<sup>1</sup> higher than the first; and the more permanent froth will collect in the trap compartment F and flow over the second lip G<sup>1</sup> into a launder H and

in most cases it will be found that the froth passing into the launder will carry the cleanest concentrate.

Any suitable means may be employed for removing the mineral from the trap compartment. If the mineral is not a clean concentrate or if it contains mixed minerals it may be re-treated conveniently in an apparatus similar to the one just described. It will be seen that the apparatus can be made in an extremely compact form as the pulp remains substantially on the same level throughout.

The apparatus affords a solution of many problems. There are many ores which are poor in sulfids, or which do not readily froth or which form a froth which is tender. The tendency in such cases is for the bubbles to break as the froth reaches the surface of the pulp and for part of the mineral to sink back into the pulp. With some frothing agents it is quite possible to get the mineral to the surface but a permanent froth is not usually formed but by the use of the apparatus embodying this invention substantially all the mineral which is floated is collected. With the frothing apparatus at present in use the froth does not have an opportunity of separating until the pulp as a whole has undergone a certain period of agitation. With some frothing agents the normal agitation is too long that is to say mineral-bearing froth formed during the commencement of the agitation is destroyed again before the froth has an opportunity of separating. With the present apparatus however the froth will come off and be trapped immediately after it is formed.

Another important problem was to provide a plant which will lend itself to the separation of the different metalliferous constituents of an ore by differential flotation. In the patent to Greenway and Lavers, No. 1,064,728, of June 17, 1913, is described a process of obtaining successive mineral bearing froths and by conducting the mixing operation under varying conditions and thereafter treating the different froths again under differentiating conditions. The apparatus embodying this invention affords ready means for carrying out such a process as the froth may be trapped, re-treated and trapped again exactly at the stages required for differentiating between the different floatable constituents.

The details of the apparatus may be varied without departing from this invention, thus the form of the conduit through which the froth passes away from the pulp may be widely varied as such conduit may be formed by suitably directed baffles, walls, tubes and the like.

The method of conveying the mineral

from the trap compartment may be by spitz-luten, by continuous water flow, by positive conveyer, by automatic valve or otherwise.

What we claim as our invention and desire to secure by Letters Patent is:—

1. A method of concentrating ores by the formation of a mineral-bearing froth which consists in causing the froth as it is formed to pass over a lip below the level of the free air surface, causing the body of the pulp to pass onward to further treatment without passing over said lip, and causing the more permanent froth of the froth thus separated to pass over a second lip.

2. A method of concentrating ores by the formation of a mineral bearing froth which consists in agitating an ore pulp mixture to aerate the same, leading off the agitated and aerated mixture and entrapping the froth as it is formed and separating the froth from the mixture before the bubbles can reach a free air surface and burst, and further separating the more permanent froth from the froth which was entrapped as it was formed.

3. A method of concentrating ores which consists in mixing the ore with water containing a mineral-frothing agent, agitating the mixture so as to beat air into it leading off the agitated and aerated mixture in which a froth forms, deflecting or guiding the froth as it rises, entrapping the froth as it forms and separating the froth from the liquid before the bubbles can reach a free air surface and burst, and further separating the more permanent froth from the froth which was entrapped as it was formed.

4. In an apparatus for concentrating ores by gaseous flotation of certain mineral particles in liquid, the combination of a vessel having agitation froth forming means, a conduit leading from the froth forming vessel to convey the liquid and the froth which forms therein, a trap to catch the froth before the bubbles reach the surface, and an overflow lip for the more permanent froth of the froth thus entrapped.

5. In an apparatus for concentrating ores by gaseous flotation of certain mineral particles in liquid, the combination of a vessel having agitation froth forming means, means forming an outlet passage leading therefrom, and a lip in the wall of said passage which is below the free air surface and over which the froth passes, whereby the froth is collected and removed before the bubbles can burst.

6. In an apparatus for concentrating ores by gaseous flotation of certain mineral particles in liquid, the combination of a vessel having agitation froth forming means, means forming an outlet passage leading therefrom, such passage-forming means hav-

ing a wall the top of which is below the free air surface and over which the froth passes, a trap compartment to receive said froth, and means for separating the more permanent froth in said trap compartment.

7. In an apparatus for concentrating ores by gaseous flotation of certain mineral particles in liquid, the combination of a plurality of vessels having agitation froth forming means and arranged substantially on the same level, means forming passageways outside the vessels connecting each vessel with the next adjacent vessel, and a froth trap at each passageway, whereby the froth formed at each stage of the agitation is led away and trapped before the bubbles reach a free air surface while the pulp passes through the series of froth-forming vessels.

8. In an apparatus for concentrating ores by gaseous flotation of certain mineral particles in liquid, the combination of a vessel having agitation froth forming means, means forming an outlet passage therefrom, a partition in the passage and a roof over the passage to lead the froth formed in the passage over the lip or partition before the bubbles get to a free air surface.

9. In an apparatus for concentrating ores by gaseous flotation of certain mineral particles in liquid, the combination of a vessel having agitation froth forming means, means forming an outlet passageway therefrom, a partition in said passageway having a lip below the free air surface in said passage, a roof to lead the froth over the lip before the bubbles get to a free air surface, a second lip over which the more permanent froth passes, and a launder on the other side of said second lip.

10. In an apparatus for concentrating ores by gaseous flotation of certain mineral particles in liquid, the combination of a plurality of vessels having agitation froth forming means, means forming connecting passages between said froth forming vessels, and froth traps in said connecting passages arranged to trap the bubbles before they reach a free air surface.

In testimony whereof we have signed our names to this specification in the presence of two subscribing witnesses.

EDWARD HOIT NUTTER.  
THEODORE JESSE HOOVER.

Two witnesses to the signature of Edward Hoit Nutter:

C. L. M. NOBLE,  
M. I. LAWRENCE.

Two witnesses to the signature of Theodore Jesse Hoover:

O. J. WORTH,  
R. C. TREDWELL.